

Dec. 6, 1938.

A. G. BOUHUYS

2,138,954

## MANUFACTURE OF ARTIFICIAL SILK HOSE

Filed Oct. 16, 1936

2 Sheets-Sheet 1



Inventor

*Aleidus G. Bouhuys*

By Albin F. Knight  
Attorney

Dec. 6, 1938.

A. G. BOUHUYS

2,138,954

MANUFACTURE OF ARTIFICIAL SILK HOSE

Filed Oct. 16, 1936

2 Sheets-Sheet 2

Fig. 5.



Fig. 6.



Fig. 7.



Inventor

Aleidus G. Bouhuys

By Albin F. Knight  
Attorney

## UNITED STATES PATENT OFFICE

2,138,954

## MANUFACTURE OF ARTIFICIAL SILK HOSE

Aleidus G. Bouhuys, Enka, N. C., assignor to  
 American Enka Corporation, Enka, N. C., a corporation of Delaware

Application October 16, 1936, Serial No. 106,035

3 Claims. (Cl. 66—178)

This invention relates to fabric formed primarily of artificial silk yarn, and more specifically to a knitted fabric formed of artificial silk yarn composed primarily of yarns having different lustres.

Artificial silk fabrics have to a large extent replaced natural silk fabrics particularly in those instances where high gloss effects are desired such as in the production of draperies and the like. However, in the manufacture of hosiery and other wearing apparel artificial silk yarn has not met with the same demand as it has in other fields because of certain objections thereto. One of the objections to the use of artificial silk yarn in the manufacture of hosiery was that normal artificial silk yarn presented an objectionable high gloss when used for this purpose. Methods have now been devised for the production of delustered and partly delustered artificial silk yarn, and millions of pounds of such yarn are produced annually in the United States. Such delustered yarn has to a limited extent replaced natural silk yarn in the manufacture of hosiery, but it has been found that such replacement of natural silk yarn by low lustre artificial silk yarn has been made possible only because artificial silk yarn was sold at a rate considerably below the price of natural silk yarn.

It is now generally recognized that hosiery produced from the better grades of artificial silk yarn compares favorably with hosiery made of natural silk yarn from the standpoint of dye affinity, wearing characteristics and the like. However, in view of the historical development of the hosiery art, natural silk hosiery has continued to be in great demand and to be thought of as being the preferred hosiery, particularly since natural silk hosiery presents a glittering effect as compared with artificial silk hosiery. So far as I am aware, attempts to produce fabrics and particularly artificial silk hosiery which present the glittering effect comparable with natural silk hosiery have been unsuccessful, and it is this feature in particular to which my present invention is directed.

It is an object of the present invention to produce a composite artificial silk yarn, which when manufactured into fabric will present a glittering effect, while maintaining in the yarn and fabric the advantages normally present therein. Additionally, this invention contemplates the production of a knitted fabric which is capable of being freely stretched and uniformly dyed with freedom from streaks or rings, and which presents the glittering effect characteristic of natural silk fabric irrespective of the dye with which it is impregnated.

A further object of this invention is the production of a composite artificial silk yarn from a multiplicity of high lustre filaments and a multi-

plicity of low lustre filaments in which the low lustre filaments and the high lustre filaments are independently extruded, coagulated and stretched and are then collected together either on a bobbin or within a centrifugal pot or bucket. After collection, the filaments are subjected to the usual treating operations involved in the manufacture of artificial silk yarn. In case the freshly spun filaments are collected and treated on a bobbin, they are later twisted in the normal manner on a twisting bobbin. If the filaments are collected in a centrifugal bucket, they receive the desired twist normally imparted by the rotation of the bucket.

This invention, however, further contemplates the individual collection of the high lustre filaments and the low lustre filaments on separate bobbins or in separate pots. If collected on separate bobbins, the composite yarn may be later formed and twisted by means of the so-called ring twister. Naturally, the collection in separate pots provides for a twisted yarn of low lustre and a twisted yarn of high lustre. These twisted yarns of different lustres may then be twisted together to form the composite yarn.

Other objects and advantages of the invention will be apparent from the following detailed description when considered in connection with the accompanying drawings wherein:

Figure 1 illustrates diagrammatically a separate extrusion of low lustre filaments and high lustre filaments into the same spinning bath and means for bringing together in parallel relationship the different lustered filaments and collecting the same in an untwisted condition on a bobbin;

Figure 2 is illustrative of the so-called "up-twister" wherein the low lustre filaments and high lustre filaments collected on the bobbin in Figure 1 are rewound and twisted together on a twisting bobbin;

Figure 3 illustrates diagrammatically a mechanism for the individual extrusion of high lustre filaments and low lustre filaments into the same spinning bath including means for individual conveyance thereof and collection upon separate bobbins;

Figure 4 illustrates a ring-twister on which the yarns produced by the mechanism illustrated in Figure 3 are twisted to form a composite yarn;

Figure 5 illustrates diagrammatically a mechanism for the independent extrusion into the same spinning bath of low lustre filaments and high lustre filaments, and the separate withdrawing and conveying means for the filaments, together with a centrifugal spinning bucket for collecting the composite yarn and twisting the same by centrifugal force developed from rotation of the said bucket;

Figure 6 is similar to Figure 5 except that the

low lustre filaments and the high lustre filaments have common withdrawing and conveying means, and

Figure 7 represents an enlarged section of 5 knitted fabric such as that formed on the usual type of hosiery knitting machine, the fabric being knitted from the composite yarn produced by the mechanism shown in Figures 1 and 2, Figures 3 and 4, Figure 5 or Figure 6.

10 Referring to the drawings in detail and particularly to Figure 1, a spinneret 10 is arranged below the surface of a coagulating bath 11 for the extrusion of a plurality of delustered cellulosic filaments 12 into the said coagulating bath 11. 15 These filaments 12 are passed through the coagulating bath 11 and led over a thread guide 13 to and around a godet wheel 14. The filaments may be passed one or more times around the godet wheel after which they are directed to an idle 20 roller 15. From the idle roller 15 the filaments comprising the yarn body are passed through a traverse guide 16 and collected upon a bobbin 17 in the usual manner. A spinneret 10a similar to spinneret 10 is arranged in a side by side relationship below the surface of the coagulating bath 11 for the extrusion of undelustered or lustrous filaments 12a into the said coagulating bath. The filaments comprising the yarn body 12a are passed over a thread guide 13a and thence to 25 the godet wheel 14 over which the filaments 12 are being passed concurrently. The high lustre filaments 12a and the low lustre filaments 12 may be brought together as they are passed over the godet wheel 14 one or more times, or they may 30 be maintained separate by means of the thread guides 13a and 13 respectively. By means of the godet wheel 14 the filaments 12a are conveyed along with the filaments 12 to the aforementioned idle roller 15, whereafter the untwisted high 35 lustre and low lustre filaments are collected on the bobbin 17 after they have passed through the traverse guide 16.

The bobbin 17 preferably rotates at a peripheral speed higher than the peripheral speed 40 of the godet wheel 14 whereby tension is placed upon the filaments between the bobbin and godet wheel. This imparts a predetermined amount of stretch to the filaments at this stage of the process. The godet wheel 14 is positively driven by 45 any suitable means, not shown, the peripheral speed of which is changed during the spinning operation in order to increase the stretch on the filaments according to the teachings of the Thurmond Patent No. 2,076,801. This procedure is 50 desirable during the period of formation and collection of the yarns in order to enhance the dyeing qualities thereof, as more fully set forth in the foregoing Thurmond patent.

The high lustre and low lustre yarn collected on 55 the bobbin 17 may now be treated in the usual way; for instance, it may be subjected to the normal treatments including desulphurizing, washing, bleaching and drying. After having been processed, the untwisted yarn is conveyed 60 by means of a suitable support 18 (see Figure 2) to a position whereby the yarns can be readily twisted. The yarns 19 are passed through a ring guide 20 and a traverse guide 21 to a twisting bobbin 22 and the high lustre and low lustre 65 70 yarns are thereby combined and twisted to form a composite body.

Referring to Figure 3 of the drawings, spinnerets 23 and 24 are shown immersed in a spinning bath 25 for extruding a high lustre spinning 75 solution and a low lustre spinning solution there-

from respectively in a manner similar to that shown in Figure 1. The filaments forming the yarn bodies 26 and 27 are in this case withdrawn from the spinning bath 25 by means of separate godet wheels 28 and 29. The yarns 26 and 27 are 5 thereafter led around idle rollers 30 and 31 respectively to be ultimately collected in untwisted condition on bobbins 32 and 33. In collecting the high lustre filaments and the low lustre filaments 10 separately as distinguished from the mechanism shown in Figure 1 the speeds of the godet wheels and the bobbins are controlled and maintained similar to the godet wheel and bobbin exemplified in Figure 1.

After the usual processing and drying the un- 15 twisted yarn bodies are each conveyed to a position in advance of a ring twister 34, as shown in Figure 4, and twisted to form a composite yarn.

Figures 5 and 6 exemplify mechanisms for producing composite yarns according to the centrifugal spinning method. In first referring to Figure 5, a spinneret is shown at 35 immersed in a coagulating bath 36. A low lustre cellulosic solution is forced through the spinneret 35 by means of a pump, not shown, and the resultant 20 filaments forming a yarn 37 are passed through the coagulating bath and led around a godet wheel 38. In the form shown the filaments 37 are caused to pass one or more times around the godet wheel 38 and are then conducted to a second godet wheel 39. The filaments are also caused to pass one or more times around this godet wheel 39 and are then directed over an idle roller 40. Another spinneret 41 is immersed adjacent the spinneret 35 in the spinning bath 36 25 and an undelustered or high lustre cellulosic solution is forced through the openings in the spinneret 41 whereupon the resultant filaments 42 are conducted to a godet wheel 43 and led therearound one or more times. The filaments 42 pass 30 from the godet wheel 43 to a second godet wheel 44 and wound thereabout one or more times. From the said godet wheel 44 the filaments are 35 passed over an idler roller 45. The godet wheels 38, 39, 43 and 44 are positively driven by any 40 suitable means, not shown, the peripheral speeds of the godet wheels 38 and 43 being maintained uniform with respect to each other while the peripheral speeds of the godet wheels 39 and 44 are maintained the same with respect to each 45 other. However, the godet wheels 39 and 44 are 50 operated at greater peripheral speeds than the respective godet wheels 38 and 43 whereby a stretching action is imparted to both the low lustre filaments 37 and the high lustre filaments 55 42 during the spinning operation. It is preferable to change the speeds of the respective sets of the godet wheels while the yarn passes therebetween in accordance with the disclosure of the Thurmond patent referred to above. This permits the formation and collection of the yarns under a gradually increasing stretch in order to 60 improve the dyeing properties.

The groups of filaments 37 and 42, as they are 65 passed over the respective idle rollers 40 and 45 are directed into contact with each other and passed down through a vertically reciprocating funnel guide 46, whereupon, due to the action of a rapidly rotating spinning bucket 47, the 70 respective groups of filaments are spun and twisted into a composite yarn by means of the centrifugal force developed from the rotation of the said bucket. The composite yarn is deposited within the bucket 47 in the form of a yarn cake 48. The cake 48 may now be subjected to the usual treat- 75

ments including desulphurizing, washing, bleaching and drying.

Referring more particularly to Figure 6, high lustre and low lustre filaments are extruded from the spinnerets 49 and 50 in a similar manner as described with respect to Figure 5. These groups of filaments 51 and 52 are maintained separate by means of thread guides 53 and 54 respectively during their passage to the same godet wheel 55 and are thereafter led around this godet wheel 55 to a second godet wheel 56 and thence to an idle roller 57. During the concurrent travel of the high lustre filaments and the low lustre filaments over the godet wheels and the idle roller, the groups of filaments may be maintained separate or brought together. The groups of filaments are finally directed downwardly through a spinning funnel 58 and collected in spinning bucket 59 to produce a yarn cake 60 in the same manner as that described in connection with Figure 5.

The source of cellulosic solutions supplied to the spinnerets shown in Figures 1, 3, 5 and 6 may be located at any convenient point. In supplying high lustre and low lustre cellulosic solutions the spinning machines comprising a plurality of spinning positions may be fitted out with independent position feed lines arranged parallel to each other and adapted for feeding alternate spinning positions with high lustre solutions and low lustre solutions respectively.

The twisted composite yarns produced in accordance with the procedures outlined in Figures 1 to 6 inclusive are now in condition for forming into a fabric. The composite yarn may be dyed either before or after it is formed into a fabric.

In the manufacture of hosiery the knitted fabric is normally in the form shown in Figure 7. It has been found that those portions of the composite yarn body which present glossy exterior surfaces when knitted into the fabric will so reflect the light as to cause the fabric to present a glittering effect or glints probably due to the existence of a dull lustre surface which interrupts the otherwise continuous lustrous effect. It is to be understood that such effect may also be attained in woven fabrics.

As a specific example of one complete process in which hosiery has been produced in accordance with the present invention, a viscose solution was prepared in the usual manner so as to have a viscosity of 7,000 centipoises, a cellulose content of 7.5% and a caustic soda content of 7%. The spinning solution was ripened to a sodium chloride index of Hottenroth maturity of 10 c. c. (see Reinthal and Rowe, "Artificial Silk" 1928, page 68).

The viscose was delivered to a 30 hole spinneret at the rate of 6 grams per minute and extruded therethrough into a coagulating bath heated to 42° C., having approximately the following composition:

| Per cent       |      |
|----------------|------|
| Sulphuric acid | 10.0 |
| Sodium sulfate | 18.0 |
| Zinc sulfate   | 1.5  |
| Glucose        | 6.0  |
| Water          | 64.5 |

The filaments were led to and passed completely around a driven godet wheel having an initial peripheral speed of 60 meters per minute then to another godet wheel having a peripheral speed of 70 meters per minute. The filaments were then led over an idle roller and to a spinning pot. A second viscose solution of substantially the same composition as that described with the ad-

dition of 10.0% pine oil and 1.2% titanium dioxide calculated on the weight of cellulose content in the viscose to constitute a delustering agent was prepared and extruded through a 30 hole spinneret at the rate of 6 grams per minute into the same coagulating bath. The filaments were led to and around two godet wheels in series and then over an idle roller as described in connection with the lustrous filaments aforesaid.

The two groups of filaments or yarn bodies were contacted at a point subsequent to their passage over the idle rollers and directed by means of a vertically reciprocating funnel guide into a spinning pot rotating at the rate of approximately 8,000 R. P. M. The passage of the yarn bodies into the pot rotating at 8,000 R. P. M. at the rate of 70 meters per minute caused the composite yarn to be twisted to a low twist of 3 turns to the inch. The cake was doffed from the bucket, wrapped in cheesecloth and washed with soft water in the usual manner and dried. The dried cake was processed in the well known manner for desulphurizing, bleaching and dyeing the yarn.

The thus prepared yarn was used in a conventional knitting machine for the fabrication of stockings in the usual way. Hosiery prepared from the yarn above described was found to present the glittering effect characteristic of the better class hosiery knitted from natural silk.

As another specific example of a complete process in which hosiery has been produced in accordance with the present invention, viscose was prepared in the usual manner so as to have a viscosity of 7,000 centipoises, a cellulose content of 7.5% and a caustic soda content of 7%. The spinning solution was ripened to a sodium chloride index of 10 c. c. according to Hottenroth.

The viscose was delivered to a 30 hole spinneret at the rate of 6 grams per minute and extruded therethrough into a coagulating bath heated to 42° C., having the following composition:

| Per cent       |      |
|----------------|------|
| Sulphuric acid | 10.0 |
| Sodium sulfate | 18.0 |
| Zinc sulfate   | 1.5  |
| Glucose        | 6.0  |
| Water          | 64.5 |

The filaments were led to and around a godet wheel and over an idle roller in the manner described above.

A second viscose solution was prepared and extruded in a similar manner except that to the spinning solution there was added titanium dioxide to the extent of 1.2% of the total solution as a delustering agent.

The two groups of filaments or yarn bodies were collected on the same bobbin in the manner illustrated in Figure 1. The yarns were washed, desulphurized, bleached, dyed and dried in accordance with the usual procedure and passed to an up-twister, which formed the yarns or group of filaments into a single composite yarn having a twist of 5 turns per inch. The spools of yarn were coned or reeled into skeins and used in a standard machine for knitting hosiery and the hosiery produced was found to present the glittering effect characteristics of hosiery fabricated from natural silk yarn.

It has been found that a composite yarn produced in accordance with this invention when twisted from 3 to 5 turns per inch produces the most satisfactory results on yarns when the yarns

are formed in accordance with the specific examples above described. The respective godet wheels in the first specific example referred to were operated so that the peripheral speeds of the first godets in the paths of travel of the filaments were 60 meters per minute and the peripheral speeds of the second respective godets were 70 meters per minute. During the spinning operation the speeds of the second godets were increased to 75 meters per minute and in this way the yarn bodies were increasingly elongated as they were collected in the respective buckets or pots. In the second specific example the godet wheel was operated so that the peripheral speed was 65 meters per minute and the peripheral speed of the bobbin was 70 meters per minute. During the spinning period the peripheral speed of the bobbin was increased to 71.5 meters per minute and in this way the yarns were increasingly stretched to effect uniform dyeing thereof.

The glittering effect referred to above is noted when the fabric is viewed at an angle to its surface. When hosiery formed from natural silk yarn is viewed in such a way that the angle between the line of sight and the surface of the fabric is an acute angle (preferably less than 45°), the surface of the hosiery presents a glittering effect which is apparently due to the light being reflected from a large number of small surfaces, having the appearance of points. Hosiery formed of artificial silk yarn prepared from filaments of uniform lustre presents a dull monotonous gloss lacking the glittering appearance characteristic of hosiery formed of natural silk yarn. Hosiery formed and other fabrics formed of yarn prepared in accordance with the present invention are seen to possess the same glittering appearance that is noted in connection with fabrics formed of natural silk yarn. The similarity is so marked that fabrics formed of natural silk yarn cannot be differentiated from those formed of artificial silk yarn prepared in accordance with the present invention by ordinary visual inspection.

Whereas the apparatus and process have been described as applied to the drawings, various other modifications and changes may be made to fall within the scope of the invention.

What I claim is:

1. A process of producing knitted hose from viscose thread which, when so formed, presents a glittering effect similar to that presented by a knitted natural silk hose which comprises extruding a viscose solution containing a deluster-

ing material to produce delustered filaments, passing the filaments through a coagulating bath, extruding a normal viscose solution to produce lustrous filaments, passing said filaments through the same coagulating bath, stretching the respective filaments from a common source and propelling the filaments to a point of collection, twisting the said filaments together 3 to 5 turns per inch, knitting the composite thread into hose so that lustrous portions of the thread occur which are of such size and so spaced that a glittering effect and a degree of luster similar to that of knitted natural silk hose is presented.

2. A process of producing hose knitted from viscose thread which, when so formed, presents a glittering effect similar to that presented to knitted natural silk hose which comprises concurrently extruding a normal viscose solution and a viscose solution containing a delustering material through the same coagulating bath to produce a group of lustrous filaments and a group of delustered filaments, withdrawing and propelling the two groups of filaments in side by side relationship from the bath by a common draw-off means and collecting the filaments on a bobbin, processing and drying in package form the untwisted filaments, twisting the two groups of filaments to obtain a low twist and form a single thread, and knitting the thread into hose so that lusterous portions of the thread occur which are of such size and so spaced that a glittering effect and a degree of lustre similar to that of knitted natural silk hose is presented.

3. A process of producing hose knitted from viscose thread which, when so formed, presents a glittering effect similar to that presented to knitted natural silk hose which comprises concurrently extruding a normal viscose solution and a viscose solution containing a delustering material through the same coagulating bath to produce a group of lustrous filaments and a group of delustered filaments, withdrawing and propelling the two groups of filaments in side by side relationship from the bath by a common draw-off means and collecting the filaments in a centrifugal bucket, processing and drying in package form the twisted thread, and knitting the thread into hose so that lusterous portions of the thread occur which are of such size and so spaced that a glittering effect and a degree of lustre similar to that of knitted natural silk hose is presented.

ALEIDUS G. BOUHUYS.